

March 23, 1943.

D. J. CAMPBELL

2,314,342

PRODUCING ARTILLERY PROJECTILE BODIES

Filed March 18, 1941

4 Sheets-Sheet 1

FIG. 1.



FIG. 2.



Donald J. Campbell Inventor

Charles W. Dake  
Attorney

March 23, 1943.

D. J. CAMPBELL

2,314,342

PRODUCING ARTILLERY PROJECTILE BODIES

Filed March 18, 1941

4 Sheets-Sheet 2

FIG. 2.



Donald J. Campbell <sup>Inventor</sup>  
By

Charles W. Dake

Attorney

March 23, 1943.

D. J. CAMPBELL

2,314,342

PRODUCING ARTILLERY PROJECTILE BODIES

Filed March 18, 1941

4 Sheets-Sheet 3

FIG. 3.



FIG. 7.



FIG. 4



Donald J. Campbell <sup>Inventor</sup>  
By

Charles W. Dake  
Attorney

March 23, 1943.

D. J. CAMPBELL

2,314,342

PRODUCING ARTILLERY PROJECTILE BODIES

Filed March 18, 1941

4 Sheets-Sheet 4

FIG. 5.



FIG. 6.



Inventor

Donald J. Campbell

Charles W. Dake

Attorney

## UNITED STATES PATENT OFFICE

2,314,342

## PRODUCING ARTILLERY PROJECTILE BODIES

Donald J. Campbell, Spring Lake, Mich.

Application March 18, 1941, Serial No. 383,937

6 Claims. (Cl. 22—113)

My present invention relates to improvements in artillery projectile bodies having a cavity wherein to carry a charge of high explosive during its flight, and the objects of improvement are, first, to provide an artillery projectile body of cast ferrous metal; second, to provide an artillery projectile body of cast ferrous metal that will be sound and free from imperfections; third, to provide an artillery projectile body whereof the constituent structure will be uniform; fourth, to provide an artillery projectile body that will burst in chunks and not in elongated splinters as do such bodies formed from ductile steel by drawing and forging; fifth, to provide an artillery projectile body whereof the base will be sound and free from porosity; sixth, to provide a hollow artillery projectile wherein the cavity for carrying the charge of high explosive will be substantially concentric with the outer periphery of the projectile; seventh, to provide a method for producing artillery projectile bodies that will meet the above named objects; which I attain by the artillery projectile body herein described and the structure of the projectile and mold illustrated in the accompanying drawings, in which—

Figure 1 is a plan view of the mold in which four artillery projectile bodies embodying my improvements are produced, the view having line I—I designating the plane on which the following vertical sectional views are taken.

Figure 2 is a vertical sectional view of my preferred mold structure in which my projectile body is cast, the section is taken on line I—I of Figure 1, and illustrates the structure of the mold with the projectile casting cavities and arrangement of the gates and passages through which the molten ferrous metal is delivered into the casting cavities and the means for assisting in preventing porosity in the base of the projectile.

Figure 3 is a sectional view showing an alternative structure to that of Figure 2.

Figure 4 is a cross-sectional view of one of the mold units taken on line II—II, of Figure 2.

Figure 5 is a sectional view of the mold, the cores forming the cavities in the projectiles, the cavities therefor and portions of the gates for delivering molten metal to the mold cavities, the section is taken on a plane extending transversely of the mold on line III—III of Figure 2 and looking downward from said line.

Figure 6 is a similar sectional view to that of Figure 5, except it is taken on a transverse plane looking downward from line IV—IV of Figure 2,

the view shows the arrangement of the gates through which the molten metal is delivered to the mold cavities, the mold cavities in which the projectile bodies are cast and cores whereby the cavities within the projectile body is formed.

Figure 7 is an elevation view of an artillery projectile body as cast by my improved method, the projectile body having a portion cut away in order to show the cavity within the projectile.

Figure 8 is a vertical cross-sectional view of the insert for preventing porosity in the base portion of the projectile body, and for supporting the core forming the cavity within the projectile.

Throughout the drawings similar numerals refer to similar parts or portions; and referring thereto:

Numeral 1 represents a projectile casting of ferrous metal such as steel and cast in my chill mold which consists of a lower portion 2 comprising a plurality of chill portions 3 and upper mold portion 4 comprising a plurality of chill portions 5, or the alternate structure shown in Figure 3, which has a plurality of sand portions 6 within the flask portion 7 which is shown provided with a plurality of outwardly extending lugs 7a having holes extending therethrough for the reception of flask pins 7b that are supported by lugs 7c, extending outward from the lower mold portion 3. In my preferred mold, the upper portion rests on and is separated from the lower mold portion 3 by core like slab 8 having a plurality of gates 9 extending to the mold cavities 10, from gate ring cavity 11 which is connected to runner sprue cavity 12 connected to the gate ring cavity 11, and to the sprue cavity 13 by vertically disposed gates 14, the sprue cavity terminates at its lower end into basin 13a. Each mold cavity 10 has supported therein core portion 15 and guide portion 15a both built of granular core material around perforated hollow arbor 16 supported at its top by key 17 extending through the arbor at its upper end and through the neck 18 of the mold. The cores 15 and 15a are further supported by insert member 19 which consists of a base plate 2, having a downward extending lug 21, inverted L cross-sectional segmental annularly formed collar 22, cup like portion 23 engaging the lower extremity of the core 15 and neck 24 for supporting the cup 23 and thereby the core 15.

Artillery projectile bodies at present are usually produced in the rough by a forging process in which lengths of cylindrical steel billets are heated to a high forging temperature and upset to

form a somewhat flat wad or body of steel which is again heated to a like forging temperature, placed between drawing dies mounted in a powerful press and drawn or forged to the shape of a large elongated shell having a closed end and another end open to permit withdrawal of the punch portion of the dies, and after the forging has been removed from the dies and cooled, it is machined both exteriorly and interiorly, the machined forging is then again heated and its open end swaged to form the conical front portion of the projectile and thickened to permit cutting a screw thread therein after which the projectile body is machined for length, the exterior finish machined and the screw threads for securing the fuse in the cut in the end of the projectile body.

Artillery projectiles produced by the process described have objections that cannot be eliminated by drawing or forging, these objections are, the constituent structure is drawn out longitudinally of the projectile, therefore is broken into elongated splinters or slivers when burst by the explosive force of the high explosive charge, and not into chunks as required, and in many cases merely expand the front end of the projectile in broom like formation and leaving the base intact with the further objections, the projectile produced by drawing or forging are expensive to produce and do not lend themselves to rapid production. These objections are entirely overcome in the projectile produced by my improved method, which consists in providing a chill mold of ferrous metal such as steel, to the form shown in the accompanying drawings, which comprises the lower portion 1 extending preferably upward to the slab core 8.

In carrying out the method of producing artillery projectile bodies, I provide the mold as shown and described. I place within each mold cavity of the mold, the insert member 19, with its under flat side resting against the bottom of the mold cavity and the cup thereof upward to engage the under end of the core 15 which is supported by the cup axially within the mold cavity, or I may suspend the core in the mold cavity as shown in Figure 2, by the key 17 extending through the arbor 16 upon which the core is built around, and having provided the mold with the core and insert member 19 therein, and having provided molten metal preferably an alloy steel, I pour into the sprue cavity 13 the said molten metal which flows downward therein and through vertically extending gates 14 into runner ring cavity 12 from where the molten metal flows into the gate ring cavity 11 and therefrom through the gates 9 to the mold cavity 10, wherein is formed the projectile body casting and in which is embedded the insert member 19 which forms an integral part of the projectile body completely fused to the metal of the projectile body. The purpose of the insert besides supporting the core in the mold, forms a seal against entrance of hot gases that might ignite the charge of high explosive within the projectile cavity, also refines the metal comprising the base portion of the projectile and further reinforces the projectile body against expansion within the gun barrel caused by the sudden force of the burning propelling explosive.

Having described my improved method for producing artillery projectile bodies and the projectile produced by the said method, the rights, I desire are set forth in the claims hereafter enumerated.

1. In producing artillery projectile bodies, the

combination comprising a mold having upper and lower portions of ferrous metal in vertically spaced apart relation and a sand core like slab interposed between said upper and lower portions of which the upper portion has a plurality of cavities in which to form the front portions of projectile bodies, the lower portion having a plurality of cavities in which to form the base portions of projectile bodies, the sand core like slab having cavities portions in which to form the intermediate portions of projectile bodies and a ring gate cavity encircling each mold cavity and having gates extending therefrom to the respective mold cavity for delivering molten metal from the said ring gate to the mold cavity formed by the said upper, lower and sand core like slab, a vertically disposed runner sprue cavity extending vertically between all of the said mold cavities and having at its lower end a plurality of vertically disposed rectangular cross-sectional gates for delivering molten metal from the said runner sprue to the ring gate cavities, a core supported in each mold cavity for forming the explosive carrying cavity and supported in said cavity by a ferrous metal member comprising a cup engaging the base of said core, a base plate extending over the bottom of the mold cavity, and a neck like support extending between the said cup and base.

2. In producing artillery projectile bodies having an explosive carrying cavity, the combination consisting of a mold having upper and lower portions of ferrous metal in vertically spaced apart relation, a sand core like slab interposed between the said portions of which the upper portion has a cavity in which to form the front portion of projectile bodies, the lower portion having a cavity in which to form the base portions of projectile bodies, the core like slab having a cavity in which to form the intermediate portion of the projectile bodies and a plurality of gates extending to the said cavities for delivering molten metal to the cavities formed by the said upper, lower and sand core like slab, a runner sprue cavity extending vertically adjacent the said cavities and having vertically disposed gates for delivering molten metal from the said runner sprue to the gate extending to the mold cavity in the said sand core like slab, a core supported in the mold cavity for forming the explosive carrying cavity and supported in said cavity by a ferrous metal member engaging the base of said core and a base engaging the bottom of the mold cavity.

3. In producing artillery projectile bodies having an explosive carrying cavity, the combination consisting of a mold comprising upper and lower portions in vertically spaced apart relation and a core like slab interposed between said upper and lower portions of which the upper portion has a cavity in which to form the front portion of the projectile body, the lower portion having a cavity in which to form the base portion of the projectile body, the core like slab having an annular cavity in which to form the intermediate portion of the projectile body and ring gate cavity encircling gates extending from the ring gate to the mold cavity for delivering molten metal from the said ring cavity to the mold gate portion formed by the said sand core like slab member, a runner sprue cavity extending vertically in spaced apart relations to the said mold cavity and having at its lower end a vertically disposed rectangular cross-sectional gate for delivering molten metal from the said runner sprue cavity to the ring gate, a core supported in the mold

cavity for forming the explosive carrying cavity therein and supported in said cavity by a ferrous metal insert comprising a cup engaging the said core, a base plate extending over the bottom of the mold cavity from the base plate and a support for the said cup extending between the cup and the said base.

4. In a mold wherein to cast projectile bodies, the said mold consisting of a lower casting chill portion in which to form the base of the projectile, an upper casting chill portion in which to form the front portion of the projectile, a core composition slab like member separating the said lower and upper portions and having therein a plurality of gates for delivering molten metal to the lower and upper chill portions, and a core support that becomes embedded into the projectile body when the said body is cast by its fusion with the metal of the body, the said core support comprising a cup for engaging the core forming 20 the projectile charge cavity and a base with a neck separating the said cup and base.

5. In a mold wherein to cast projectile bodies, a lower casting chill portion and an upper casting chill portion with a core composition member separating the said mold portions and having a hole extending therethrough in registration with the cavities of the said lower and upper mold portions and a plurality of gates therein for delivering molten metal to the said casting chill portions.

6. In a mold wherein to cast projectile bodies, an upper casting chill portion having a cavity in which to form a portion of the projectile body, a lower casting chill portion having a cavity in which to form the base portion of the projectile and having therein a core of granular core material and a cup like core supporting member engaging the end of the cavity of the lower casting chill portion and the end of the core, substantially as described.

DONALD J. CAMPBELL.